# EUROPEAN PATENT APPLICATION

(11) **EP 4 289 297 A1**
(43) Date of publication of application: **13.12.2023**
(21) Application number: 21923673.4
(22) Date of filing: 02.02.2021
(51) Int. Cl.: A24F 40/46

(54) **HEATING COMPONENT AND ELECTRONIC ATOMIZING DEVICE**

(71) Applicant: Shenzhen Smoore Technology Limited, Shenzhen, Guangdong 518102 (CN)
(72) Inventor: DUAN, Yinxiang, Shenzhen, Guangdong 518102 (CN); JIANG, Jinfeng, Shenzhen, Guangdong 518102 (CN); ZHU, Mingda, Shenzhen, Guangdong 518102 (CN); CHEN, Peng, Shenzhen, Guangdong 518102 (CN); XIE, Jiansheng, Shenzhen, Guangdong 518102 (CN); DU, Jing, Shenzhen, Guangdong 518102 (CN); BU, Guihua, Shenzhen, Guangdong 518102 (CN); ZHENG, Liangfu, Shenzhen, Guangdong 518102 (CN); XIONG, Yuming, Shenzhen, Guangdong 518102 (CN); WU, Zhenxing, Shenzhen, Guangdong 518102 (CN); FAN, Jingbo, Shenzhen, Guangdong 518102 (CN)
(74) Representative: De Arpe Tejero, Manuel
(86) International application number: PCT/CN2021/074920
(87) International publication number: WO 2022/165644

(57) **Abstract**

A heating component and an electronic atomizing device. The heating component comprises a ceramic matrix and a heating layer. The heating layer comprises stainless steel and an inorganic nonmetal, is used to heat a substrate to be atomized to form an aerosol, and has a TCR temperature-sensitive property. The inorganic non-metal is used to adjust the TCR value of the heating layer. By using the heating layer made of stainless steel, the heating component is enabled to have properties such as high-temperature resistance, high high-temperature stability, high-temperature oxidation resistance, and strong solution corrosion resistance; and by adding an inorganic non-metallic material to the stainless steel, a resistance-temperature coefficient of the heating layer is adjusted, and temperature control of the heating layer is achieved, preventing the generation of a miscellaneous gas and a burning smell during an atomization process, ensuring fragrance consistency, and helping to improve the usage experience of a user.

## Description

### TECHNICAL FIELD

The present disclosure relates to the field of atomizer technologies, in particular to a heating assembly and an electronic atomizing device.

### BACKGROUND

Most of ceramic atomizing cores of several electronic atomizing devices with a better taste on the market are made by printing on a porous ceramic substrate with iron-nickel-chromium or iron-chromium-aluminum. Iron-nickel-chromium or iron-chromium-aluminum has characteristics such as high-temperature tolerance, high stability at high temperatures, and high tolerance to high-temperature oxidation and solution corrosion.

As the technology of the electronic atomizing device becomes increasingly mature, users have a higher requirement for the taste. However, in general electronic atomizing devices, ceramic atomizing cores cannot achieve temperature control. Further, during atomization, phenomena such as a miscellaneous gas, a burning smell, and poor fragrance reduction may occur, affecting user experience.

### SUMMARY OF THE DISCLOSURE

Based on the above, the present disclosure provides a heating assembly and an electronic atomizing device to solve a technical problem that a metal layer of a ceramic atomizing core cannot realize temperature control in the related art.

In order to solve the above technical problem, a first technical solution provided in the present disclosure is to provide a heating assembly, including a ceramic substrate and a heating layer. The heating layer includes stainless steel and inorganic nonmetal. The heating layer is configured to heat an ingredient to be atomized to form an aerosol. The heating layer includes a TCR temperature-sensitive characteristic. The inorganic nonmetal is configured to adjust a value of the TCR of the heating layer.

In some embodiments, the stainless steel includes one or more of 316L stainless steel, 304 stainless steel, and 430 stainless steel.

In some embodiments, the inorganic nonmetal includes one or more of SiO₂, Al₂O₃, ZrO₂, and SiC.

In some embodiments, the Non-stainless steel metal is further included, and the non-stainless steel metal includes one or more of Mo, Ti, Zr, and Mg.

In some embodiments, a glass is further included, and the glass includes one or more of a SiO₂-ZnO-BaO system, a SiO₂-CaO-ZnO system, a SiO₂-ZnO-R₂O system, and a SiO₂-B₂O₃ system.

In some embodiments, the heating layer includes stainless steel, inorganic nonmetal, glass, and non-stainless steel metal. The stainless steel accounts for 75-85% by weight of the heating layer, the inorganic nonmetal accounts for 0.5-3% by weight of the heating layer, the glass accounts for 11.5-21.5% by weight of the heating layer, and the non-stainless steel metal accounts for 0.5%-3% by weight of the heating layer.

In some embodiments, the stainless steel is one or more of 316L stainless steel, 304 stainless steel, and 430 stainless steel. The inorganic nonmetal is one or more of SiO₂, Al₂O₃, ZrO₂, and SiC. The non-stainless steel metal is one or more of Mo, Ti, Zr, and Mg. The glass is one or more of a SiO₂-ZnO-BaO system, a SiO₂-CaO-ZnO system, a SiO₂-ZnO-R₂O system, and a SiO₂-B₂O₃ system.

In some embodiments, the thickness of the heating layer ranges from 100 µm to 120 µm. The resistance of the heating layer ranges from 0.6 S2 to 0.8 Ω.

In order to solve the above technical problem, a second technical solution provided in the present disclosure is to provide an electronic atomizing device, including a heating assembly, the heating assembly is the heating assembly according to any one described above.

Beneficial effects of the present disclosure are as follows. Different from the related art, the heating assembly in the present disclosure includes a ceramic substrate and a heating layer. The heating layer includes stainless steel and inorganic nonmetal. The heating layer is configured to heat an ingredient to be atomized to form an aerosol. The heating layer includes a TCR temperature-sensitive characteristic. The inorganic nonmetal is configured to adjust the value TCR of the heating layer. The heating layer is made of stainless steel, so that the heating assembly has characteristics such as high-temperature tolerance, high stability at high temperatures, high tolerance to high-temperature oxidation and solution corrosion. Inorganic nonmetals are added to the stainless steel to realize temperature control of the heating layer, thereby avoiding miscellaneous gas and a burning smell during atomizing, ensuring consistency of fragrance, and improving user experience.

### BRIEF DESCRIPTION OF THE DRAWINGS

In order to more clearly illustrate the technical solutions in the embodiments of the present disclosure, the accompanying drawings for describing the embodiments are briefly introduced below. Apparently, the accompanying drawings in the following description present only some embodiments of the present disclosure. For the skilled in the art, other accompanying drawings may be derived from these accompanying drawings without creative efforts.
FIG. 1 is a structural schematic view of an electronic atomizing device provided in the present disclosure.
FIG. 2 is a structural schematic view of a heating assembly provided in the present disclosure.
FIG. 3 is a scanning electron microscope image of microscopic morphology of a heating layer in a heating assembly provided in the present disclosure.
FIG. 4 is a schematic flowchart of a method to fabricate a heating assembly provided in the present disclosure.
FIG. 5 is a diagram of a relationship between resistance and temperature of heating assemblies in Experiment 7 provided in the present disclosure.

### DETAILED DESCRIPTION

The following description is a further detailed description of the present disclosure in conjunction with the accompanying drawings and embodiments. Specifically, the following embodiments are only used to illustrate the present disclosure, but are not intended to limit the scope of the present disclosure. Similarly, the following embodiments are only some rather than all of the embodiments of the present disclosure, and all other embodiments obtained by the skilled in the art without creative efforts shall fall within the protection scope of the present disclosure.

The terms "first", "second", and "third" in the present disclosure are used for descriptive purposes only, and cannot be construed as indicating or implying relative importance, or implicitly indicating a quantity of indicated technical features. Therefore, features qualified with "first", "second", or "third" may explicitly or implicitly include at least one of the features. In the description of the present disclosure, "a plurality of" means at least two, e.g., two or three, etc., unless otherwise expressly and specifically limited. All directional indications (e.g., up, down, left, right, front, back. etc.) in the embodiments of the present disclosure are only used to explain relative positional relationships, movement situations, etc., between the components in a particular attitude (as shown in the accompanying drawings). If the specific attitude is changed, the directional indications are changed accordingly. In addition, the terms "comprise", "include", and "have", and any variations thereof in the embodiments of the present disclosure are intended to cover a non-exclusive inclusion. For example, a process, method, system, product, or device including a series of steps or units is not limited to the listed steps or units, but further optionally includes steps or units that are not listed, or further optionally includes other steps or units that are intrinsic to the process, method, product, or device.

Reference to "embodiment" in the present disclosure means that particular features, structures, or characteristics described in junction with the embodiments may be included in at least one embodiment of the present disclosure. The presence of the phrase at different positions in the specification may not refer to the same embodiment, nor a separate or alternative embodiment that is mutually exclusive from other embodiments. It is understood, both explicitly and implicitly, by the skilled in the art that the embodiments described in the present disclosure may be combined with other embodiments.

Referring to FIG. 1, FIG. 1 is a structural schematic view of an electronic atomizing device provided in the present disclosure.

The electronic atomizing device may be configured to atomize liquid ingredients. The electronic atomizing device includes a atomize 1 and a power supply component 2 connected to each other.

The atomizer 1 includes a heating assembly 11 and a reservoir 12. The reservoir 12 is configured to store the ingredient to be atomized. The heating assembly 11 is configured to heat and atomize the ingredient to be atomized in the reservoir to form an aerosol that can be inhaled by a user. The atomizer 1 may be specifically configured to atomize the ingredient to be atomized and generate an aerosol for use in different fields such as medical treatment and an electronic aerosol generating device. In a specific embodiment, the atomizer 1 may be applied to the electronic aerosol atomizing device and is configured to atomize the substrate to be atomized and generate an aerosol for a smoker to inhale which is taken as an example in the following embodiments. Certainly, in other embodiments, the atomizer 1 may also be applied to a hair spray device to atomize hair spray for hair styling. Alternatively, the atomizer is applied to a medical device for treating upper and lower respiratory system diseases to atomize medical drugs.

The power supply assembly 2 includes a battery 21, a controller 22, and an airflow sensor 23. The battery 21 is configured to supply power to the atomizer 1, so that the atomizer 1 can atomize a liquid ingredient to form an aerosol. The controller 22 is configured to operate the atomizer 1. The airflow sensor 23 is configured to detect an airflow change in the electronic atomizing device, to start the electronic atomizing device.

The atomizer 1 and the power supply assembly 2 may be integrally arranged or detachably connected, which is designed according to specific needs.

Referring to FIG. 2, FIG. 2 is a structural schematic view of a heating assembly provided in the present disclosure.

The heating assembly 11 includes a ceramic substrate 13 and a heating layer 14. The ceramic substrate 13 is a porous ceramic. The ceramic substrate 13 contacts the ingredient to be atomized in the reservoir 12. The ceramic substrate guides the ingredient to the heating layer 14 by capillary force. Then, the heating layer 14 heats and atomizes the ingredient to form an aerosol. The heating layer 14 includes stainless steel and inorganic nonmetal. The heating layer 14 is configured to heat and atomize the ingredient to be atomized to form an aerosol. The heating layer 14 has a TCR (temperature coefficient of resistance) temperature-sensitive characteristic. The inorganic nonmetal is configured to adjust the value of TCR of the heating layer 14. That is, the heating layer 14 in some embodiment of the disclosure is made of stainless steel, so that the heating layer 14 has the TCR temperature-sensitive characteristic. Thus, the heating assembly 11 has the characteristics such as high-temperature tolerance, high stability at high temperatures, and high tolerance to high-temperature oxidation and solution corrosion of an existing ceramic atomizing core. Further, inorganic nonmetals are added to the heating layer 14 to adjust the value of TCR of the heating layer 14, which can realize temperature detection and control of the heating layer 14, thereby avoiding miscellaneous gas and a burnt smell during atomizing, improving a heat flux density and temperature-field uniformity of the heating assembly 11, improving consistency of fragrance, and improving user experience.

The stainless steel includes one or more of 316L stainless steel, 304 stainless steel, and 430 stainless steel, or may be stainless steel of another grade. A maximum temperature for heating and atomizing the ingredient is preferably controlled below 350 degrees. However, in general stainless steel, the value of TCR of the heating film is too high, thereby a temperature of the heating film easily exceeding 350 degrees. This problem may be solved by adding inorganic nonmetal in the present disclosure. The inorganic nonmetal includes one or more of SiO₂, Al₂O₃, ZrO₂, and SiC, or may be another inorganic nonmetal. By adding a small amount of inorganic nonmetal in the heating layer 14, the resistance, the temperature coefficient of resistance, and the corrosion resistance of the heating layer 14 may be adjusted. The stainless steel and inorganic nonmetal in the heating layer 14 may be selected according to needs, as long as the temperature of the heating assembly 11 is controllable. For example, the heating layer 14 is consisted of stainless steel and inorganic nonmetal. The inorganic nonmetal accounts for 1% of the total weight of the heating layer 14.

Further, the heating layer 14 includes non-stainless steel metal. The non-stainless steel metal includes one or more of Mo, Ti, Zr, and Mg. By adding a small amount of metal such as Mo, Ti, Zr, and Mg in the heating layer 14, the compactness and uniformity of the heating layer 14 are good, which is beneficial to improving the corrosion resistance, high-temperature resistance, and lifetime of the heating layer 14. Good compactness and uniformity of the heating layer 14 also enhance a bonding force between the heating layer 14 and the ceramic substrate 13, thereby greatly improving the electrochemical stability of the heating layer 14 in the electronic atomizing device during operation. For example, the heating layer 14 is consisted of stainless steel, non-stainless steel metal, and inorganic nonmetal. the inorganic nonmetal accounts for 1% of the total weight of the heating layer 14, and the non-stainless steel metal accounts for 0.5% of the total weight of the heating layer 14.

Currently, most of the heating layers in conventional heating assemblies are heating layers of iron-nickel-chromium or iron-chromium-aluminum printed on porous ceramic substrates. However, when a heating layer 14 with such an alloy is applied in an electronic atomizing device, heavy metal ions (such as nickel and chromium) may be detected in an ingredient to be atomized and aerosol components. It may be understood that, in the present disclosure, the electrochemical stability of the heating layer 14 in the operating environment of the electronic atomizing device is improved by adding a small amount of metal such as Mo, Ti, Zr, and Mg in the heating layer 14, so that heavy metal content in the substrate to be atomized and the aerosol is greatly reduced, thereby solving the key problem of potential safety hazards caused by existing heating assemblies to users.

In the present disclosure, the heating layer 14 is made by drying a resistance paste. The resistance paste includes stainless steel powder, non-stainless steel metal, inorganic nonmetal, glass, and organic carriers. The organic carriers include resins and solvents. In the drying process of the resistance paste, the organic carriers continue to volatilize. Therefore, the heating layer 14 is consisted of stainless steel powder, non-stainless steel metal, inorganic nonmetal, and glass. A difference between the heating layer 14 and the resistance paste lies in whether organic carriers are included or not. By adding the glass in the heating layer 14, matching between the stainless steel and the ceramic substrate 13 is enhanced, thereby improving the sintering stability of the stainless steel heating layer 14 and solving the sintering problem of the stainless steel heating layer 14.

Among them, the stainless steel powder accounts for 60%-76.5% of the total weight of the resistance paste, the glass accounts for 9.2%-17.2% of the total weight of the resistance paste, the inorganic nonmetal accounts for 0.4%-2.7% of the total weight of the resistance paste, the non-stainless steel metal accounts for 0.4%-2.7% of the total weight of the resistance paste, and the organic carriers account for 10%-20% of the total weight of the resistance paste.

The glass is a SiO₂-ZnO-BaO system. The glass system may better match the ceramic substrate 13, to prevent the ceramic substrate from being damaged by the stress generated by sintering at high temperatures, or prevent the heating layer 14 from cracking. The glass system is not limited to the SiO₂-ZnO-BaO system. Other systems such as SiO₂-CaO-ZnO, SiO₂-ZnO-R₂O, and SiO₂-B₂O₃ may also be optional in the present disclosure. The specific glass systems may be selected according to the sintering process of the ceramic substrate 13 and the resistance paste.

The organic carriers include resins and solvents. The resin includes ethyl cellulose, and the solvent includes terpineol and butyl carbitol acetate systems. Both terpineol and butyl carbitol acetate are good solvents for ethyl cellulose. A combination of terpineol and butyl carbitol acetate may control the volatility and leveling of the resistance paste. In addition, terpineol and butyl carbitol acetate may adjust the viscosity of the organic carriers. With a proper viscosity, the organic carriers may fully wet metal and inorganic nonmetal, thereby improving the printability of the resistance paste. Ethyl cellulose accounts for 3%-8% of the total weight of the organic carriers, terpineol accounts for 50%-70% of the total weight of the organic carriers, and butyl carbitol acetate accounts for 27%-42% of the total weight of the organic carrier. In other embodiments, the resin may also be cellulose acetate butyrate, acrylic resin, and polyvinyl butyral, etc. The solvent may also be butyl carbitol, diethylene glycol dibutyl ether, triethylene glycol butyl ether, alcohol ester dodeca, tributyl citrate, and tripropylene glycol butyl ether, etc. Specific material composition of the resin and solvent may be selected according to needs.

In the heating layer 14 made by drying the resistance paste, the stainless steel accounts for 75%-85% of the total weight of the heating layer 14, the glass accounts for 11.5%-21.5% of the total weight of the heating layer 14, the inorganic nonmetal accounts for 0.5%-3% of the total weight of the heating layer 14, and the non-stainless steel metal accounts for 0.5%-3% of the total weight of the heating layer 14.

Referring to FIG. 3, FIG. 3 is a scanning electron microscope image of microscopic morphology of a heating layer in a heating assembly provided in the present disclosure.

In the present disclosure, a mesh panel used for the resistance paste printed includes 200 mesh, a yarn thickness of 80 µm, an emulsion thickness of 100 µm, and a line width of 0.5 mm for printing. With the mesh panel, the heating layer 14 is obtained after drying and sintering. The microscopic morphology is shown in FIG. 3. The thickness of the heating layer 14 ranges from 100 µm to 200 µm, and the resistance ranges from 0.6 S2 to 0.8 S2. In other embodiments, spraying, physical vapor deposition (PVD), chemical vapor deposition (CVD), and other processes may also be used to fabricate the heating layer 14. The specific process may be selected according to needs.

Referring to FIG. 4, FIG. 4 is a schematic flowchart of a method to fabricate a heating assembly provided in the present disclosure. The method for fabricating the heating assembly 11 includes the following operations.

At operation S01, the method may include obtaining a ceramic substrate.

Specifically, S01 includes preparing ceramic powder and obtaining the ceramic substrate 13 through a process such as screen printing or sintering, etc.

At operation S02, the method may include forming a heating layer on a surface of the ceramic substrate.

Specifically, S02 includes preparing resistance paste with raw materials used to form the heating layer 14; printing the resistance paste on the surface of the porous ceramic substrate 13 through mesh panel; forming the heating layer 14 on a surface of the ceramic substrate 13 through drying and sintering the ceramic substrate 13 and the resistance paste at 1000-1250 °C.

In an embodiment, in the resistance paste, the stainless steel powder accounts for 75% of the total weight of the resistance paste, the glass accounts for 12% of the total weight of the resistance paste, the inorganic nonmetal accounts for 1% of the total weight of the resistance paste, the non-stainless steel metal accounts for 0.5% of the total weight of the resistance paste, and the organic carriers account for 11.5% of the total weight of the resistance paste. In the organic carriers, the resin accounts for 5% of the total weight of the organic carriers, and the solvent accounts for 95% of the total weight of the organic carriers. The thickness of the heating layer 14 is 100 µm, and the resistance is 0.6 Ω.

The stainless steel powder adopts 361L stainless steel powder, the glass adopts a SiO₂-ZnO-BaO system, the inorganic nonmetal adopts SiO₂, the non-stainless steel metal adopts Mo and Mg, the resin in the organic carriers adopts ethyl cellulose, and the solvent adopts terpineol and butyl carbitol acetate systems. Ethyl cellulose accounts for 5% of the total weight of the organic carriers, terpineol accounts for 60% of the total weight of the organic carriers, and butyl carbitol acetate accounts for 35% of the total weight of the organic carriers.

It may be understood that pins need to be arranged on the heating layer 14 of the heating assembly 11 to be electrically connected to the battery 21 The pins are coated with silver paste to prevent the pins from being corroded by a substrate to be atomized or a atomized aerosol, to play a role of protecting. Another metal coating may also be selected, according to needs, to protect the pins.

The heating assembly 11 provided in the present disclosure is compared with the first existing heating assembly (No.1), and the performance is proved through experiments. The heating assembly 11 provided in the present disclosure for the experiment is consists of stainless steel, non-stainless steel metal, glass, and inorganic nonmetal. The stainless steel adopts 361L stainless steel powder, the glass adopts a SiO₂-ZnO-BaO system, the inorganic nonmetal adopts SiC, and the non-stainless steel metal adopts Mo or Mg. Stainless steel accounts for 75% by weight of the heating layer, inorganic nonmetal accounts for 1% by weight of the heating layer, glass accounts for 12% by weight of the heating layer, and non-stainless steel metal accounts for 0.5% by weight of the heating layer. The main component of a heating layer in a first heating assembly (No.1), which is existing in general use, is nickel-chromium (T29) with a nickel-chromium content of 85.6% and a glass content of 14.4%. For the convenience of statistics, the heating assembly 11 provided in the present disclosure is recorded as a second heating assembly (No.2).

### Experiment 1: Test for lifetime in dry combustion cycle

Experimental conditions: Constant power of 6.5 W, on-state for 3 seconds and off-state for 8 seconds, and 50 times for cycles.

The heating assembly 11 provided in the present disclosure and the first heating assembly (No.1) were tested under the above experimental conditions to determine a resistance change and whether the resistance change is invalid. In order to ensure the accuracy of experimental results, three parallel experiments were performed on the heating assembly 11 in the present disclosure and the first heating assembly (No.1). The experimental results are shown in Table 1.

**Table 1: Test for lifetime of 316L stainless steel heating layer in dry combustion**

| Heating assembly | Quantity of cycles/time | Invalid or not | Resistance change | Test environment |
|---|---|---|---|---|
| No. 1 | 10 | Yes | Invalid | Air |
| No. 1 | 13 | Yes | Invalid | Air |
| No. 1 | 11 | Yes | Invalid | Air |
| No. 2 | 50 | No | No change | Air |
| No. 2 | 50 | No | 0.02 Ω | Air |
| No. 2 | 50 | No | 0.01 Ω | Air |

### Experiment 2: Test for lifetime in wet combustion cycle

Experimental conditions: Constant power of 6.5 W, on-state for 3 seconds and off-state for 8 seconds, and 400 times for cycles.

The heating assembly 11 provided in the present disclosure and the first heating assembly (No.1) were tested under the above experimental conditions to determine a resistance change and whether the resistance change is invalid. In order to ensure the accuracy of the experimental results, three parallel experiments were performed on the heating assembly 11 in the present disclosure and the first heating assembly (No.1). Experimental results are shown in Table 2.

**Table 2: Test for lifetime of 316L stainless steel heating layer in wet combustion**

| Heating assembly | Quantity of cycles/time | Break or not | Resistance change | Test environment |
|---|---|---|---|---|
| No. 1 | 400 | No break | No change, but the surface turns black | Glycerol |
| No. 1 | 400 | No break | No change, but the surface turns black | Glycerol |
| No. 1 | 400 | No break | No change, but the surface turns black | Glycerol |
| No. 2 | 400 | No break | No change, and no blackening | Glycerol |
| No. 2 | 400 | No break | No change, and no blackening | Glycerol |
| No. 2 | 400 | No break | No change, and no blackening | Glycerol |

### Experiment 3: Metal dissolution test in 4% acetic acid

Experimental conditions: Soak in 4% acetic acid.

The heating assembly 11 provided in the present disclosure and the first heating assembly (No.1) were tested under the above experimental conditions, and amounts of metal dissolution were compared. Experimental results are shown in Table 3.

**Table 3: 4% acetic acid soaking results**

| Heating assembly | Amount of leached Ni (g/ml) | Amount of leached Cr (g/ml) |
|---|---|---|
| No. 1 | 16.2 | 1.1 |
| No. 2 | 0.093 | 0.033 |

### Experiment 4: Metal dissolution test in mango e-liquid of 57 mg

Experimental conditions: Soak in mango e-liquid of 57 mg.

The heating assembly 11 provided in the present disclosure and the first heating assembly (No.1) were tested under the above experimental conditions, and amounts of metal dissolution were compared. Experimental results are shown in Table 4.

**Table 4: Soaking results of mango e-liquid of 57 mg**

| Heating assembly | Amount of leached Ni (g/ml) | Amount of leached Cr (g/ml) |
|---|---|---|
| No. 1 | 3.0 | 1.0 |
| No. 2 | 0.08 | 0.03 |

### Experiment 5: Heavy metal content in flue gas

Experimental conditions: Mango e-liquid of 57 mg, constant power of 6.5 W, inhaling for 3S and stopping for 8S, and inhalation of 100 puffs.

The heating assembly 11 provided in the present disclosure and the first heating assembly (No.1) were tested under the above experimental conditions, and heavy metal contents in the flue gas were compared. Experimental results are shown in Table 5.

**Table 5: Heavy metal content in flue gas**

| Heating assembly | Ni content in flue gas (g/100 puffs) | Cr content in flue gas (g/100 puffs) |
|---|---|---|
| No. 1 | 2.542 | 0.138 |
| No. 2 | Not detected | Not detected |

### Experiment 6: Film-base bonding force

A bonding force between the heating layer 14 and the ceramic substrate 13 in the heating assembly 11 provided in the present disclosure and a bonding force between a heating layer and a ceramic substrate in the first heating assembly (No.1) were tested, and film-base bonding forces were compared. Experimental results are shown in Table 6.

**Table 6: Film-base bonding force test results**

| Heating assembly | Thrust value/gf |
|---|---|
| No. 1 | 1700 |
| No. 2 | 2100 |

### Experiment 7: Test for temperature coefficient of resistance

Temperature coefficients of resistance (TCR) of heating layers and ceramic substrates in the heating assembly 11 provided in the present disclosure, the first heating assembly (No. 1), and a third heating assembly (No.3), which is existing in general use, were tested. The main component of the heating layer of the third heating assembly (No.3) is stainless steel. A relationship between the resistance and temperatures of the second heating assembly (No.2) and the third heating assembly (No.3) is shown in FIG. 5 (FIG. 5 shows a relationship between resistance and temperature of heating assemblies in Experiment 7 according to the present disclosure). Calculation results are shown in Table 7.

**Table 7: Temperature coefficient of resistance (TCR)**

| Heating assembly | TCR (ppm/°C) |
|---|---|
| No. 1 | / |
| No. 2 | 726 |
| No. 3 | 1067 |

As can be seen from the experimental results in Table 1 and Table 2, the lifetime of the heating assembly 11 (the second heating assembly (No.2)) provided in the present disclosure is longer than that of the first heating assembly (No.1). As can be seen from the experimental results in Table 3, Table 4, and Table 5, metal ion dissolution of the heating assembly 11 (the second heating assembly (No.2)) provided in the present disclosure is two orders of magnitude lower than that of the first heating assembly (No.1), and heavy metal cannot be detected in the flue gas. Therefore, the heating assembly 11 provided in the present disclosure may significantly reduce potential safety hazards caused by the material of the heating layer 14 to the user. As can be seen from the experimental results in Table 6, a film-based bonding force of the heating assembly 11 provided in the present disclosure (the second heating assembly (No.2)) is higher than that of the first heating assembly (No.1), which indicates that the heating assembly 11 has better physical shock resistance. As can be seen from the experimental results in Table 7, compared with the first heating assembly (No.1), the heating assembly 11 (the second heating assembly (No.2)) provided in the present disclosure has TCR performance and can realize temperature control of the heating layer 14, thereby reducing miscellaneous gas and a burning smell. In addition, by adding inorganic nonmetal, the value of TCR of the heating layer 14 may be effectively changed, the lifetime of the heating assembly 11 is prolonged, the heat flux density and the temperature field uniformity of the heating layer 14 are improved, and taste consistency and user experience are improved.

The heating assembly in the present disclosure includes a ceramic substrate and a heating layer. The heating layer includes stainless steel and inorganic nonmetal. The heating layer is configured to heat a substrate to be atomized to form an aerosol. The heating layer includes TCR temperature-sensitive characteristic. The inorganic nonmetal is configured to adjust the value of TCR of the heating layer. The heating layer is made of stainless steel, so that the heating assembly has characteristics such as high-temperature tolerance, high stability at high temperatures, and high tolerance to high-temperature oxidation and solution corrosion. Inorganic nonmetals are added to the stainless steel to realize temperature control of the heating layer, thereby avoiding miscellaneous gas and a burning smell during atomizing, ensuring consistency of fragrance, and improving user experience.

The above descriptions are only some embodiments of the present disclosure, and the protection scope of the present disclosure is not limited thereto. All equivalent apparatus or process changes made according to the content of the specification and accompanying drawings in the present disclosure or by directly or indirectly applying the present disclosure in other related technical fields shall fall within the protection scope of the present disclosure.

## Claims

1. A heating assembly, applied to an electronic atomizing device, and comprising:
a ceramic substrate; and
a heating layer, comprising stainless steel and inorganic nonmetal, wherein the heating layer is configured to heat an ingredient to be atomized to form an aerosol; the heating layer features a, temperature coefficient of resistance, TCR, and the inorganic nonmetal is configured to adjust the value of the TCR of the heating layer.

2. The heating assembly as claimed in claim 1, wherein the stainless steel comprises one or more of 316L stainless steel, 304 stainless steel, and 430 stainless steel.

3. The heating assembly as claimed in claim 1, wherein the inorganic nonmetal comprises one or more of SiO₂, Al₂O₃, ZrO₂, and SiC.

4. The heating assembly as claimed in claim 1, further comprising non-stainless steel metal, wherein the non-stainless steel metal comprises one or more of Mo, Ti, Zr, and Mg.

5. The heating assembly as claimed in claim 4, further comprising glass, wherein the glass comprises one or more of a SiO₂-ZnO-BaO system, a SiO₂-CaO-ZnO system, a SiO₂-ZnO-R₂O system, and a SiO₂-B₂O₃ system.

6. The heating assembly as claimed in claim 5, wherein the heating layer is consisted of the stainless steel, the inorganic nonmetal, the glass and the non-stainless steel metal; the stainless steel accounts for 75-85% by weight of the heating layer; the inorganic nonmetal accounts for 0.5-3% by weight of the heating layer; the glass accounts for 11.5-21.5% by weight of the heating layer; and the non-stainless steel metal accounts for 0.5-3% by weight of the heating layer.

7. The heating assembly as claimed in claim 6, wherein the stainless steel is one or more of 316L stainless steel, 304 stainless steel, and 430 stainless steel; the inorganic nonmetal is one or more of SiO₂, Al₂O₃, ZrO₂, and SiC; the non-stainless steel metal is one or more of Mo, Ti, Zr, and Mg; and the glass is one or more of the SiO₂-ZnO-BaO system, the SiO₂-CaO-ZnO system, the SiO₂-ZnO-R₂O system, and the SiO₂-B₂O₃ system.

8. The heating assembly as claimed in claim 1, wherein the thickness of the heating layer ranges from 100 µm to 120 µm.

9. The heating assembly as claimed in claim 1, wherein the resistance of the heating layer ranges from 0.6 S2 to 0.8 Ω.

10. An electronic atomizing device, comprising a heating assembly, wherein the heating assembly is the heating assembly as claimed in any one of claims 1 to 9.
